

## UNITED STATES PATENT OFFICE

2,110,491

## PHOTOGRAPHIC EMULSIONS

Marti Salo, Rochester, N. Y., assignor, by mesne assignments, to Eastman Kodak Company, Jersey City, N. J., a corporation of New Jersey

No Drawing. Application April 16, 1936,  
Serial No. 74,815

15 Claims. (Cl. 95—7)

This invention relates to photographic emulsions and particularly to emulsions in which a hydrolyzed cellulose ester is used as the protective colloid for the light-sensitive salt.

5 Various substances have been suggested and tried as carriers or protective colloids for the light-sensitive salts used in photography, but, as is well-known, none has been found which possess the unique chemical and physical properties of gelatin. Collodion was used for this purpose before the discovery of the useful properties of gelatin as a photographic carrier and even up to the present time, it is used in certain commercial processes. Two methods of processing 10 photographic plates were developed, namely, the dry and the wet process. According to the first method, the light sensitive halides were precipitated in an alcohol-ether solution of collodion which was then coated onto a glass or other support and exposed and processed in a manner similar to the present gelatin procedure. The second process involves treating an iodized collodion plate in a silver nitrate bath immediately prior to exposure and development.

15 Of these two early processes employing collodion, only the wet plate process has continued to be of any importance. One objection to the collodion process is the low water permeability of cellulose nitrate films. Coincident with this 20 is the insolubility of cellulose nitrate in solvent mixtures containing appreciable amounts of water, which consequently prevents the use of water-soluble salts such as the common alkali halides used in forming the light-sensitive halides of the present gelatin process.

25 The use of cellulose acetate as a carrier for light-sensitive salts, has also been suggested. Eichengrun U. S. Patent No. 752,388, February 16, 1904, suggested alcohol solutions of cellulose acetate, and Lederer British Patent No. 26,503 of 1906 suggested cellulose acetates soluble in acetic acid as carriers of light-sensitive salts. Up to the present time, however, photographic emulsions formed in this way have not been 30 successful and have not gone into general use.

35 The principal object of the present invention is to provide a carrier or protective colloid for light-sensitive silver salts which has the physical and photographic properties of gelatin.

40 This object is accomplished according to the present invention by dispersing silver halides in the presence of a water-susceptible, hydrolyzed, mono-basic, simple or mixed acid ester of cellulose.

45 55 It is known that cellulose acetate and other

mono-basic simple and mixed cellulose esters may be hydrolyzed and that as the degree of hydrolysis increases, the esters become soluble in the more polar types of solvents such as 1,4 dioxane, beta-methoxy-ethyl alcohol and ethyl lactate. On further hydrolysis a stage is reached where these esters become soluble in solvent mixtures containing as much as 50% water.

5 On account of the presence of appreciable amounts of water, a solvent mixture such as 10 ethyl lactate and water will dissolve the hydrolyzed cellulose ester and will also dissolve appreciable quantities of inorganic salts such as sodium chloride, sodium bromide, silver nitrate, etc. It is therefore possible to precipitate a light-sensitive halide such as silver bromide in the 15 colloidal dispersion of the cellulose ester, somewhat similar to the manner in which the silver bromide is dispersed in gelatin. On coating a 20 solution containing the silver halide suspended in the hydrolyzed cellulose ester onto a suitable support, there is obtained a light-sensitive coating which may be used to record photographic images.

25 The cellulose esters which may be used as protective colloids for the light-sensitive salts according to my invention, include the mono-basic simple and mixed acid esters of cellulose such as cellulose acetate, cellulose acetate propionate, cellulose acetate butyrate and others. 30 These are hydrolyzed to an acyl content of about 19 to about 33%. Hydrolyzed esters having an acyl content of 19 to 26% are particularly useful, due to their high water permeability. The hydrolyzed esters used according to my invention have been prepared prior to the present invention. Esters hydrolyzed to an acyl content of about 30% are described in Staud and Webster U. S. Patents No. 1,896,145, granted February 7, 1933, and No. 1,954,336, granted April 10, 1934. 40 Cellulose esters hydrolyzed to an acyl content of below 30% are described in the co-pending application of Charles R. Fordyce Serial No. 62,333, filed February 4, 1936.

45 As stated above, the solubility of the cellulose esters in various solvents changes as the degree of hydrolysis is increased. In order to form a dispersion of light-sensitive inorganic salts in the hydrolyzed cellulose ester solution, it is necessary to use a solvent-water mixture which 50 dissolves both the cellulose ester and the inorganic salts used to precipitate the light-sensitive salt. On the basis of hydrolyzed cellulose acetate as a criterion, the following solvent-water mixtures have been found suitable:

Hydrolyzed cellulose acetate of 33% acetyl is soluble as follows:

|                           | Percent by weight<br>water in mixture |
|---------------------------|---------------------------------------|
| 6 Acetone + water         | 5-40                                  |
| 1,4-dioxane + water       | 0-50                                  |
| Methyl-cellosolve + water | 0-25                                  |
| Ethyl lactate + water     | 0-50                                  |

Hydrolyzed cellulose acetate of 19 to 26% acetyl  
10 is soluble as follows:

|                              | Percent by weight<br>water in mixture |
|------------------------------|---------------------------------------|
| Acetone + water              | 35-80                                 |
| Ethyl lactate + water        | 35-70                                 |
| 15 Methyl cellosolve + water | 20-65                                 |
| 1,4 dioxane + water          | 30-65                                 |
| Ethyl alcohol + water        | 40-70                                 |
| n-propyl alcohol + water     | 50-80                                 |

20 The following examples illustrate methods of forming a light-sensitive coating according to my invention:

#### Example I

25 A solution of 1.9 grams of potassium bromide in 5 cc. of a 1:1 ethyl lactate-water mixture was mixed with a solution containing 3 grams of cellulose acetate hydrolyzed to an acetyl content of about 33% dissolved in 21 grams of a solvent mixture containing 75% ethyl lactate and 25% water. 30 To this was then added slowly with good stirring, a solution of 2.9 grams of silver nitrate dissolved in 5 cc. of a 1:1 solution of ethyl lactate and water. Finely divided silver bromide was thereby produced in suspension in the solution.

35 After diluting with 20 cc. of 1:1 ethyl lactate-water, the emulsion was poured slowly into 200 to 300 cc. of water causing the acetate and the occluded salts to be precipitated. The precipitated material was thoroughly washed with water 40 and then dried in an air drier, following which the dried material was dissolved in a solvent consisting of 54.5% ethylene chloride, 27.2 methyl alcohol and 18.3% beta-methoxyethyl alcohol, one part of the dried material being dissolved in 45 10 parts of the solvent mixture. This solution was then coated onto a glass plate in a uniform coating of approximately .001" thick.

The plate was exposed to light and then immersed in a developing bath of the following 50 composition:

| Water                                 | cc.   | 500  |
|---------------------------------------|-------|------|
| Monomethyl p-aminophenol sulf-<br>ate | grams | 3.1  |
| 55 Sodium sulphite                    | do    | 45.0 |
| Hydroquinone                          | do    | 12.0 |
| Sodium carbonate                      | do    | 67.5 |
| Potassium bromide                     | do    | 1.9  |
| Water to make                         | liter | 1    |

#### Example II

60 A solution of 6.6 grams of potassium bromide dissolved in 32 grams of a 1:1 ethyl lactate-water mixture was mixed with a solution containing 9 grams of cellulose acetate butyrate hydrolyzed to an acetyl content of 27% and butyryl content of 4.5% in 111 grams of a solvent mixture composed of an ethyl lactate-water mixture in the proportion of 6 parts of ethyl lactate to 4 parts of water. 65 70 8.5 grams of silver nitrate dissolved in 20 grams in a 1:1 ethyl lactate-water mixture were added with good stirring. To this emulsion there were then added 9 grams of the cellulose acetate butyrate dissolved in 111 grams of 6:4 ethyl lactate-water solution.

This emulsion was coated onto baryta coated paper in an even coating of approximately .001" thick and exposed in a contact printer using average negatives. The paper carrying the emulsion was then placed in a developing solution having the following composition:

|                                       |       |      |
|---------------------------------------|-------|------|
| Water                                 | cc.   | 500  |
| Monomethyl p-aminophenol sulf-<br>ate | grams | 3.1  |
| Sodium sulphite                       | do    | 45.0 |
| Hydroquinone                          | do    | 12.2 |
| Sodium carbonate                      | do    | 67.5 |
| Potassium bromide                     | do    | 1.9  |
| Water to make                         | liter | 1    |

The penetration of the developer was found to be slow, but when the developer was diluted 1:1 with water, the penetration was much more rapid. The addition of ethyl carbamate to the developer in the amount of 20 grams of ethyl carbamate 20 to 100 cc. of developer and 100 cc. of water was found to further increase the rate of penetration of developer. The prints were fixed for ten minutes in a bath containing 10 grams of sodium thiosulfate and 5 grams of potassium thiocyanate dissolved in 50 cc. of water. It was found that the potassium thiocyanate, in addition to being a solvent for the silver halide, served as a swelling agent for the hydrolyzed esters and thereby accelerated the fixing process.

#### Example III

25 A solution of 4.2 grams of potassium bromide in a mixture of 5 cc. of beta-methoxyethyl alcohol and 9 cc. of water was added to a solution containing 6 grams of cellulose acetate hydrolyzed to an acetyl content of about 24.4% in 21.6 cc. of beta-methoxymethyl alcohol and 14.4 cc. of water. 30 35 40 45 5.4 grams of silver nitrate dissolved in 9 cc. of water and 5 cc. of beta-methoxyethyl alcohol were then added with good stirring and silver bromide precipitated in the solution.

This emulsion was coated on baryta paper, as before, and exposed and developed. Good results were obtained when the developer used in Example II was diluted with 4 parts of water.

Emulsions formed from hydrolyzed cellulose esters, as described above have numerous advantages over ordinary gelatin emulsions. They have good mechanical strength and are not so liable to breaking and rupturing in processing. They are insoluble in water and thereby permit higher temperature baths to be used in processing, as is frequently required in tropical photographic work. Emulsions formed in this way also have the advantage that greater uniformity may be obtained in their manufacture.

The compounds and methods of procedure described above may be varied within wide limits. Although I have found that the cellulose esters containing 19 to 24% acyl are most suitable for the process of my invention due to their favorable water susceptibility, emulsions may be made with cellulose esters having a greater acyl content even though the water susceptibility of these emulsions is less favorable. A lower limit of 19% has been placed on the acyl value of the hydrolyzed esters. This is an approximate value, since esters of slightly lower acyl content may be used in applications where the water solubility is not a hindrance. Because of this water solubility, however, cellulose acetates of less than 19% acetyl would not find wide practical application. It is to be understood that my invention is limited only by the scope of the appended claims.

I claim:

1. The method of making a sensitive photographic emulsion which comprises dispersing a silver halide in a solution of a hydrolyzed cellulose organic acid ester of approximately 19% to approximately 33% acyl content.
2. The method of making a sensitive photographic emulsion which comprises dispersing a silver halide in a solution of a hydrolyzed cellulose mixed organic acid ester of approximately 19% to approximately 33% acyl content.
3. The method of making a sensitive photographic emulsion which comprises dispersing a silver halide in a solution of hydrolyzed cellulose acetate butyrate of approximately 19% to approximately 33% acyl content.
4. The method of making a sensitive photographic emulsion which comprises dispersing a silver halide in a solution of hydrolyzed cellulose acetate of approximately 19% to approximately 33% acyl content.
5. A sensitive photographic emulsion comprising a silver halide dispersed in a hydrolyzed cellulose organic acid ester of approximately 19% to approximately 33% acyl content.
6. A sensitive photographic emulsion comprising a silver halide dispersed in a hydrolyzed cellulose mixed organic acid ester of approximately 19% to approximately 33% acyl content.
7. A sensitive photographic emulsion comprising a silver halide dispersed in hydrolyzed cellulose acetate butyrate of approximately 19% to approximately 33% acyl content.
8. A sensitive photographic emulsion comprising a silver halide dispersed in hydrolyzed cellulose acetate of approximately 19% to approximately 33% acyl content.
9. The method of making a sensitive photographic emulsion which comprises dissolving a hydrolyzed cellulose organic acid ester of approximately 19% to approximately 33% acyl content.

in a solvent mixture containing approximately 50% water, dispersing a silver halide in the solution, and curing the resulting dispersion.

10. The method of making a sensitive photographic emulsion which comprises dissolving a hydrolyzed cellulose organic acid ester of approximately 19% to approximately 33% acyl content in a solvent mixture containing approximately 50% water, dispersing a silver halide in the solution, washing the excess salts from the dispersion with water, redissolving the cellulosic material containing the silver halide in a solvent-water mixture, and curing the resulting dispersion.

11. A sensitive photographic emulsion comprising a silver halide dispersed in hydrolyzed cellulose acetate having an acetyl content of 19% to 26%.

12. The method of making a sensitive photographic emulsion which comprises dispersing a silver halide in hydrolyzed cellulose acetate having an acetyl content of 19% to 26%.

13. The method of making a sensitive photographic emulsion which comprises dissolving hydrolyzed cellulose acetate of 19% to 26% acetyl content in a solvent mixture comprising  $\beta$ -methoxyethyl alcohol and water in approximately equal proportions, dispersing a silver halide in the solution, and curing the resulting dispersion.

14. The method of making a sensitive photographic emulsion which comprises dispersing a silver halide in hydrolyzed cellulose acetate butyrate having an acyl content of 19% to 26%.

15. The method of making a sensitive photographic emulsion which comprises dissolving hydrolyzed cellulose acetate butyrate of 19% to 26% acyl content in a solvent mixture comprising  $\beta$ -methoxyethyl alcohol and water in approximately equal proportions, dispersing a silver halide in the solution, and curing the resulting dispersion.

40  
MARTTI SALO.